

March 17, 1959

H. E. AUSTEN

2,878,463

MAGNETIC DATA STORAGE DEVICES

Filed March 22, 1956

FIG. 1



FIG. 2



FIG. 3



FIG. 4



INVENTOR

HERMAN E. AUSTEN

BY *Carl Beest*  
*Austin S. Austin*

HIS ATTORNEYS

1

2,878,463

## MAGNETIC DATA STORAGE DEVICES

Herman E. Austen, Trotwood, Ohio, assignor to The National Cash Register Company, Dayton, Ohio, a corporation of Maryland

Application March 22, 1956, Serial No. 573,283

4 Claims. (Cl. 340—174)

This invention relates to magnetic core storage and switching devices, suitable for use in magnetic core matrices of electronic calculating machines.

The devices consist of a number of closed magnetic cores supported on a self-supporting rigid non-magnetic structure, which holds them in position for easy insertion of electrical conductors by which data may be selectively entered into the device or read therefrom. A plurality of the devices may be formed into a coordinate matrix.

The rigid support for the cores preferably is an electrical conductor, and the supported cores may be arranged thereon in rows and columns to form a coordinate matrix. Such electrically conductive continuous rigid support may act as one of the electrical conductors in the matrix system by reason of its passing through each core.

Figs. 1, 2 and 3 show successive steps in one form of making the device, and

Fig. 4 shows a complete coordinate matrix system of two rows of the novel device.

Referring to Fig. 1, there is shown an inner support consisting of a hollow tube 10 of non-magnetic material, having closely fitted or electro-plated thereover a magnetic covering 11. The tube 10 should be of material which is rigid but which can be bent to a shape which it will retain, and, preferably of electrically conductive material, such as brass or copper.

The magnetic covering next is subjected to an operation which gives it the form of Fig. 2, as by grinding or cutting circumferential grooves at spaced intervals in the magnetic covering material until the outer surface of the support tube 10 is exposed.

Next the tube 10 is cut crosswise, at the groove intervals, the cuts being made so that the tube is held together so as to leave bridges such as 12 and 12'. As shown, the adjoining cuts are from diametrically opposite sides, leaving magnetic ring cores as individual units 13, 13'. As is known, to prevent as much as possible unwanted effects in a matrix to be made of these devices the cores in a row are alternately oriented at substantially right angles. This is done in the present invention by bending the bridges 12, 12', as shown in Fig. 4.

It is not necessary to remove the magnetic material before making the diametrically opposite cuts, as the magnetic material left on the bridges 12 would not interfere with the operation of the cores to any considerable extent.

In Fig. 4 there is shown a coordinate matrix of two rows, with five magnetic cores in each row, the matrix being shown with but few cores for the sake of simplicity. There may be as many rows and as many cores in a row as desired.

In the event the continuous supporting material 10 is an electrical conductor, adjacent rows are electrically connected, as by portion 16 of the conductor.

2

It will be seen that the rows and columns of cores shown in Fig. 4 have their holes in straight alignment as to rows and columns, so that straight electrical conductors may be strung through them with ease without bending, the supporting material serving to hold the cores without any other device being necessary, in exact spaced relation. The connector portion 16 may be of sufficient stiffness to hold the two rows of cores in proper alignment while the electrical conductors like 14 and 15 are passed therethrough.

Although the supporting tube 10 may be covered by magnetic material as by slipping over it a closely fitted tube of magnetic material, the most efficient method of covering the support is by electro-plating magnetic material thereover.

Following is the formula of a satisfactory aqueous magnetic plating solution used at 90° centigrade with a current density of 30-60 amperes per square foot:

50 grams per liter of water of  $\text{FeCl}_2 \cdot 4\text{H}_2\text{O}$   
 20 grams per liter of water of  $\text{NiCl}_2 \cdot 6\text{H}_2\text{O}$   
 12 grams per liter of water of  $\text{Na}_2\text{WO}_4 \cdot 2\text{H}_2\text{O}$   
 50 grams per liter of water of  $\text{NH}_4\text{Cl}$   
 120 grams per liter of water of Citric acid ( $\text{C}_6\text{H}_8\text{O}_7 \cdot \text{H}_2\text{O}$ )  
 1/10 gram per liter of water of thiourea  
 25 adjusted to pH 8.5 with  $\text{NH}_4\text{OH}$

The plating may be carried on until the desired thickness is obtained.

It is within the scope of the invention to form the 30 tubular support into the connected rings and then to magnetically plate them.

What is claimed is:

1. A series of closed magnetic ring-like cores each supported internally on an electrically-conductive ring, 35 the ring-supported cores of a series being arranged in a line with adjacent cores of the series having their axes at right angles, whereby an electric conductor may be easily passed through the series; and an electrically-conductive means rigidly connecting adjacent rings in alignment and orientation whereby the supporting rings and connections constitute a further conductor extending through the series of cores.

2. A series of closed magnetic ring-like cores each supported internally on an electrically-conductive ring, 45 the ring-supported cores of a series being arranged in a line with adjacent cores of the series having their axes at right angles, whereby an electric conductor may be easily passed through the series; and a bent rigid electrically-conductive means connecting adjacent rings in 50 alignment and in the right angle orientation, whereby the supporting rings and connections constitute a further conductor extending through the series of cores.

3. A series of closed magnetic ring-like cores each supported internally on an electrically-conductive ring, the 55 ring-supported cores of a series being arranged in a line, whereby to provide a straight path to enable an electric conductor to be easily passed through the series; and an angular electrically-conductive bridge rigidly connecting each two adjacent rings of the series to position adjacent 60 rings of the series with their axes at right angles, the bridges from any ring to adjacent rings extending from diametrically opposite points on a ring, said supporting rings and connecting bridges constituting a further conductor extending through the series of cores.

4. A self-supported array of rows and columns of 65 closed magnetic cores all supported on a continuous rigid framework of serially connected parallel and aligned rows of electrically conductive material which passes through each core, and to which conductive material the cores are closely fitted, the axes of adjacent cores 70 in a row being at right angles so that an electric wire may be passed in a straight line directly through the

cores of the row without bending, while magnetic induction between the cores of a row is reduced to a minimum by reason of the alternate angular position of the cores.

2,700,150 Wales Jan. 18, 1955  
 2,732,542 Minnick Jan. 24, 1956  
 2,792,563 Rajchman May 14, 1957  
 2,825,046 Herbert et al. Feb. 25, 1958

**References Cited in the file of this patent**

**UNITED STATES PATENTS**

2,278,744 Sparrow et al. Apr. 7, 1942  
 2,531,820 Lindenblad Nov. 28, 1950 10  
 2,671,950 Sukacev Mar. 16, 1954

**OTHER REFERENCES**

"Electronics," for April 1953, the front cover illustration and the illustration at the bottom of page 146 of the article entitled, "Ferrite Speed Digital Computers" by D. R. Brown and E. Albeir-Shoenberg. Pages 146 to 149.